

**United States Patent [19]****Kosaka****[11] Patent Number: 4,757,047****[45] Date of Patent: Jul. 12, 1988****[54] SUBLIMATION-TYPE THERMAL  
TRANSFER IMAGE RECEIVING PAPER****[75] Inventor: Takao Kosaka, Himeji, Japan****[73] Assignee: Mitsubishi Paper Mills, Ltd., Tokyo,  
Japan****[21] Appl. No. 895,431****[22] Filed: Aug. 11, 1986****[30] Foreign Application Priority Data**

Aug. 12, 1985 [JP] Japan ..... 60-178363

**[51] Int. Cl. 4 B41M 5/035; B41M 5/26****[52] U.S. Cl. 503;227; 8/471;  
428/342; 428/481; 428/913****[58] Field of Search 8/470, 471; 428/195,  
428/480, 913, 914, 342, 481; 430/945; 503/227****[56]****References Cited****U.S. PATENT DOCUMENTS**4,054,712 10/1977 Nagashima et al. ..... 428/481  
4,474,859 10/1984 Oshima et al. ..... 428/913  
4,490,435 12/1985 Oshima et al. ..... 8/471**FOREIGN PATENT DOCUMENTS**

0212394 10/1985 Japan ..... 428/195

*Primary Examiner*—Bruce H. Hess*Attorney, Agent, or Firm*—Cushman, Darby & Cushman**[57]****ABSTRACT**

A higher fatty acid amide(s) is(are) additionally contained in the image receiving layer containing a saturated polyester of a sublimation type thermal transfer image receiving paper. This makes it possible to obtain a uniform printed image with improved color density.

**5 Claims, No Drawings**

**SUBLIMATION-TYPE THERMAL TRANSFER  
IMAGE RECEIVING PAPER**

**TECHNICAL FIELD**

This invention relates to a sublimation type thermal transfer image receiving paper. More particularly, it relates to a sublimation type thermal transfer image receiving paper suited for use in a sublimation type thermal transfer recording system for obtaining a recorded image by heating the coloring materials on a thin support by a thermal head or other means and thereby sublimating and transferring said coloring materials.

**PRIOR ART**

According to the sublimation type thermal transfer recording system, a coloring material sheet made by applying the sublimable coloring materials on a thin support such as paper is placed in opposition to a thermal transfer image receiving paper and said sheet is heated by a thermal head for effecting color development and transfer of said coloring materials to thereby obtain a recorded image on the image receiving paper.

It is possible to obtain full-color hard copies by adopting the colors of yellow, magenta, cyan and if necessary black for the respective coloring materials and successively heating and transferring them. As the image receiving paper used in such recording system, it is known to form such paper by providing a coating layer containing a saturated polyester on a support as for instance disclosed in Japanese Patent Kokai (Laid-Open) No. 107885/82.

It is possible with this recording system to obtain a high-quality image of excellent color tone, but according to this system, since the sublimable coloring materials are sublimated directly, a large amount of heating energy is required for sublimating the coloring materials and well satisfactory color density is not obtained by use of an image receiving paper made by simply providing a coating layer containing a saturated polyester on a support.

It is therefore an object of this invention to provide a sublimation type thermal transfer image receiving paper improved in color forming characteristics.

**DISCLOSURE OF THE INVENTION**

The object of the present invention can be attained by further incorporating a higher fatty acid amide in the saturated polyester-containing layer of a sublimation type thermal transfer image receiving paper.

**DETAILED DESCRIPTION OF THE  
INVENTION**

The higher fatty acid amides usable in this invention include, for example, stearic acid amide, palmitic acid amide, oleic acid amide, methylolated stearoamide, ethylenebisstearoamide, methylenebisstearoamide, and the like. These amides may be used in combination or as a mixture.

Use of such higher fatty acid amide(s) in a too small amount proves to be ineffective, while use thereof in an excess amount may deteriorate the color forming characteristics of the produced paper due to the diluting effect. It is thus recommended to use said higher fatty acid amide(s) in an amount of 50 to 300% by weight,

preferably 80 to 200% by weight, based on the saturated polyester.

The saturated polyester used in this invention is a linear high-molecular saturated polyester formed by condensation polymerization of a dibasic acid and a dihydric alcohol. A typical example of such polyester is polyethylene terephthalate obtained by polycondensing terephthalic acid and ethylene glycol. It is also possible to use a saturated polyester made by randomly copolymerizing two or more different materials with said dibasic acid and dihydric alcohol for the improvements of crystallinity, melting point, solubility, etc.

Among other examples of said saturated polyesters are polybutylene terephthalate and poly-1,4-cyclohexanedimethylene-ethylene terephthalate. These polyesters may be used in the form of an organic solvent solution, but it is preferred to use them as a water dispersion from the viewpoint of industrial productivity. It is also desirable to use a water-soluble polyester such as a copolymer polyester of a carboxylic acid mixed with a sulfonated phthalic acid isomer and ethylene glycol.

The sublimable coloring materials used in this invention are preferably those having a sublimation point in the range of 70° to 400° C., more preferably 150° to 250° C. Examples of such sublimable coloring materials are disperse dyes such as disperse blue 20 (available under the trade name of "Duranol Blue 2G"), disperse yellow 42 ("Resulin Yellow GR"), disperse red 1 ("Celiton Scarlet B"), etc., quinalizarin dyes, dispersible monoazo dyes, dispersible anthraquinone dyes, dispersible nitrophenylamine dyes, and anthracene dyes.

As the support of said sublimable coloring materials, it is recommended to use a thin sheet or tissue-like article which has as high a heat conductivity as possible for the effective heat transfer from the thermal head. Papers such as condenser paper, grassine paper, etc., synthetic paper, synthetic resin film and the like can be used as said support. Synthetic resin film is preferred in terms of uniformity of image quality.

Fine particles of inorganic materials such as silica, calcium carbonate, kaolin, clay, colloidal silica, etc., may be added to the support for preventing heat fusion between the coloring material sheet and the image receiving paper.

The amount of the inorganic particles that can be added to the support is preferably from 25 to 100% by weight based on the total amount of saturated polyester and higher fatty acid amide(s). If the amount of said inorganic particles added is less than 25% in said weight ratio, their effect of preventing heat fusion between coloring material sheet and image receiving paper is unsatisfactory. Also, the stability of movement of the produced sheet and its releasability from the image receiving paper prove unsatisfactory. Further, it tends to occur that the desired thermal transfer of the heat-sublimated dye alone is not effected but the whole of the image receiving layer is transferred. If the amount of said inorganic particles added exceeds 100% by weight, no betterment of the heat fusion preventive effect is given and rather the color density is reduced.

In the preparation of the coloring material sheet, an adhesive having no likelihood of hindering sublimation is used. It is made into an ink, and a dye sheet can be formed by gravure printing or other means.

The support of the image receiving layer used in this invention should be one which has a good surface smoothness and a moderate degree of cushioning properties for close attachment to the thermal head. Ordin-



1. A sublimation type thermal transfer recording system comprising:
  - an image receiving paper; and
  - a coloring material sheet having a layer of heat-sublimable coloring materials, said image receiving layer being provided on a support containing a saturated polyester and one or more higher fatty acid amides.
2. The image receiving paper of claim 1, wherein the higher fatty acid amide(s) is contained in an amount of 50 to 300% by weight based on the saturated polyester.
3. The image receiving paper of claim 2, wherein the image receiving layer further contains the fine particles

- of at least one inorganic material selected from the group consisting of silica, kaolin, calcium carbonate, clay and colloidal silica.
4. The image receiving paper of claim 3, wherein the fine particles of at least one of said inorganic materials are contained in an amount of 25 to 100% by weight based on the total amount of said higher fatty acid amide(s) and saturated polyester.
5. The image receiving paper of claim 4, wherein the coating weight of the image receiving layer is 2 to 5 g/m<sup>2</sup> on the bone dry basis.

\* \* \* \* \*

15

20

25

30

35

40

45

50

55

60

65